

Dec. 19, 1950

G. C. COX

2,534,234

ELECTROCOATING METHOD

Original Filed March 7, 1947

2 Sheets-Sheet 1

Fig. 1.



Fig. 2.



INVENTOR.

George C. Cox  
BY  
Harry M. Saragovitz  
ATTORNEY

Dec. 19, 1950

G. C. COX

2,534,234

ELECTROCOATING METHOD

Original Filed March 7, 1947

2 Sheets-Sheet 2

*Fig. 3.*



*Fig. 4.*



*Fig. 5.*



Inventor

George C. Cox

By *William D. Hall.*

Attorney

## UNITED STATES PATENT OFFICE

2,534,234

## ELECTROCOATING METHOD

George C. Cox, Charleston, W. Va.

Continuation of application Serial No. 733,213,  
March 7, 1947. This application February 20,  
1948, Serial No. 9,933

7 Claims. (Cl. 204—56)

(Granted under the act of March 3, 1883, as  
amended April 30, 1928, 370 O. G. 757)

1

This invention may be manufactured and used by or for the Government for governmental purposes, without the payment to me of any royalty thereon.

This invention relates to coating methods and more particularly to the methods of electrocoating from an electrolyte which has been formed from the alkaline-earth metal salts, particularly their chlorides, sulphates or nitrates.

This invention is an improvement over the invention disclosed and claimed in my Patent Number 2,200,469 issued May 14, 1940.

It is an object of my invention to provide a novel method for producing a corrosion resistant binary coating of substantially uniform thickness.

Another object of my invention is the production of binary dielectric coatings upon objects such as wires, rods, plates, metal foils and the like.

Still another object of my invention is the production of a two component corrosion resistant coating of a non-metallic nature upon metallic surfaces, one component of which is crystalline and one amorphous.

Still another object of my invention is the production of binary coatings which may be hardened in an extremely short period of time.

The above and other objects and advantages will become readily apparent when the following specification is read in conjunction with the accompanying drawings wherein:

Figure 1 is a schematic view of an apparatus that may be utilized for carrying out my invention.

Figure 2 represents a series of graphs showing various operating conditions of my electrocoating method.

Figure 3 represents a highly magnified cross-sectional view of a coating formed under conditions to produce a high calcium content.

Figure 4 represents a highly magnified cross-sectional view of a coating formed under conditions to produce a high magnesium content.

Figure 5 represents a highly magnified cross-sectional view of a coating formed in accordance with my invention.

My method may be carried out by the use of either a large or small body of electrolyte. In general, the electrolyte used is one containing magnesium and calcium salts of the chlorides, sulphates or nitrates with or without similar salts of the alkali metals. The magnesium and calcium concentration of the electrolyte may vary from only slight salinity, such as found in

brackish waters, upward to include the concentrations found in sea water and even more concentrated solutions so that a binary non-metallic coating as hereinafter described will be formed by electrolysis within the temperature and current density ranges herein set forth.

Excellent, firmly adherent, non-metallic protecting coatings have been formed from an electrolyte of sea water or of concentrated sea water when operating at current densities above  $1/10$  ampere per square foot and under conditions delineated by the curves A to E of Fig. 2. Therefore by use of sea water or the brines made from inland salt deposits (which have been formed from sea water) an inexpensive source of raw materials is available at almost any location throughout the world. The usual mixing and replacement costs inherent in such electroplating processes is also eliminated. Various lakes have concentrated brines which can be used as a source of raw materials.

It appears that the salts of the alkaline-earth metals are essential to the formation of these two component coatings. Extremely dense coatings having excellent adherent properties have been formed from aqueous solutions of magnesium and calcium salts of the chlorides, sulphates or nitrates. Various mixtures of these salts may also be used provided that the electrolyte contains magnesium and calcium ions in sufficient quantity to cause the desired plating action to take place. It appears that the essential formation of a colloidal bonding agent is dependent upon the presence of magnesium ions in solution in sufficient quantity for the initial deposition of a gel type of matrix. The hardness of a coating appears to depend to a large extent on the quantity of the calcium ions which are discharged from solution. The ductility of an electro-deposited coating is considerably improved by the presence of ions of the alkalies such as obtained by the addition of sodium or potassium chlorides, sulphates, nitrates, etc. The hydrogen ion concentration can be varied over quite wide ranges, for example, useful coatings have been deposited from synthetic sea water and similar electrolytes of the chlorides, sulphates or nitrates of the alkaline earth metals with pH ranges as low as 4.0 and as high as 9.5. However, some of the coatings with the greatest density and best protective qualities have been formed at values between 4.5 and 5.5 on the pH scale, particularly, when sodium chloride was added to the solution. It appears that the ductility of an electro-deposited coating is improved

by the addition of sodium chloride or similar sodium salt. Furthermore the conductivity of such an electrolyte can be increased by the addition of a sodium or potassium salt such as a chloride, sulphate or nitrate.

The compounds which have been crystallized out of sea water from the various oceans are approximately:

|                           | Gms. per liter |
|---------------------------|----------------|
| Sodium chloride, about    | 26.5           |
| Magnesium chloride, about | 3.2            |
| Magnesium sulphate, about | 2.1            |
| Calcium sulphate, about   | 1.4            |
| Other salts, possibly     | 1.5            |

In terms of ion content these values are approximately:

|                       | Gms. per liter |
|-----------------------|----------------|
| Sodium ions, about    | 10.5           |
| Magnesium ions, about | 1.2            |
| Calcium ions, about   | 0.41           |
| Chloride ions, about  | 18.38          |
| Sulphate ions, about  | 2.6            |

Useful coatings have been formed when substituting chloride ion equivalent to the total equivalent non-metal negative ion content.

Similarly, this total non-metal ion equivalent can be made up from other salts of the strong acids such as the sulphates or nitrates.

Whereas the process set forth in my prior Patent Number 2,200,469 required a period of time from about 24 to 72 hours to form a suitable deposit, coatings made by the process to be herein disclosed and claimed may be formed within a period of seconds to permit the efficient, economical and high speed coating of continuous wire, strip or plate. For either continuous or intermittent modern high speed coating operations it is generally desirable to use electrolytes containing the maximum quantity of magnesium ions to which is added the maximum quantity of calcium ions that will remain in solution. The use of my method permits binary coatings of a type to be more fully described to be quickly and easily applied in a manner that was impossible to attain previous to this development.

Referring to Figure 1, a tank 17 holds therein an electrolyte 10 containing magnesium, other alkaline earth ions and ions of an alkali. The object to be coated 14, is connected to a low voltage direct current source of electricity. The electrode 15 may be covered with a substance 16 such, for example, as dolomite that will react with detrimental anode products which may be liberated during the electrolysis. The tank 17 is generally heated by means of a heating element 18 such as a steam coil or other equivalent means. For automatic operation a thermostat 11 is fixed to the side of tank 17 and controls the heating unit 18 in accordance with the desired electrolyte temperature.

In carrying out my coating method, I have found that a definite critical relationship exists between the cathode current density and the temperature of the electrolyte. This relationship may be expressed by the equation

$$T = 34 \log_{10} X + C$$

wherein  $T$  is the temperature of the electrolyte in degrees centigrade,  $X$  is the cathode current density in amperes per square foot, and  $C$  is a constant within the range of 30 to 70.

As far as can be determined, the coating resulting from the utilization of an electrolyte containing magnesium and calcium ions com-

prises substantially uniformly dispersed microscopic crystals and crystal aggregates which are compounds of calcium in the substantially pure form. These crystals are embedded in an amorphous matrix which fills the microscopic voids around the crystals so that the porosity is reduced to an extremely low value. As far as can be determined, the magnesium content of this coating composition is substantially contained in the matrix in the form of various low soluble magnesium compounds as the hydroxide, oxides, oxy-chloride, or basic carbonate, etc. It appears that this matrix is an amorphous or colloidal mixture containing the magnesium compounds with or without some of the calcium constituents.

I have found that depending on the range of current density and electrolyte temperature, the deposited coating can be made to vary from a high magnesium content, gelatinous or amorphous type of coating, to a high calcium content, highly granular, crystalline type of coating. The gelatinous type of coating is unsuitable for some applications because it may be easily washed off. On the other hand the high calcium content granular type of coating may be unsuitable for some applications since the coating contains voids between the crystals that will permit corrosive substances to penetrate the coating.

Referring to Figure 2, the five curves A, B, C, D, and E represent different conditions of electrode current density and electrolyte temperature. Operating conditions outside of the area bounded by curves A and E will result in unsatisfactory coatings. Operation below the conditions of curve A will result in a gelatinous coating having a high magnesium content, the properties of which have already been described. Operating conditions above those conditions on curve E will result in a high-calcium, highly granular, crystalline type of coating, the properties of which have already been described. The area shown between curves A and E represents the operating conditions that will result in the best coatings.

Operation of my method above the curve E of Figure 2 will result in the type of coating illustrated in Figure 3. This coating consists essentially of microscopic calcium crystals deposited on the surface being coated. The calcium crystals do not completely cover the surface and there are voids and cracks with the result that portions of the surface are exposed and receive no protection. This type of coating is not useful as a corrosion resistant coating or as a dielectric.

Utilization of my method under conditions of temperature and current densities that fall below the curve A of Figure 2 results in a coating such as illustrated in Figure 4. This coating consists essentially of magnesium compounds with little or no calcium crystals therein. Such a coating when dry contains shrinkage cracks which permit portions of the surface to be exposed. Such a deposit is not useful as a corrosion resistant coating or as a dielectric.

If the conditions of temperature and current density between curves A and E of Figure 2 are utilized, a coating such as disclosed in Figure 5 will result with the best coatings resulting from operating conditions of electrolyte temperature and current density falling between the curves B and C. In this coating, there is an abundant quantity of microscopic crystals of a calcium constituent, imbedded in an amorphous matrix con-

sisting essentially of magnesium compounds. Such a coating is tough, resilient and is excellent for the purpose of providing corrosion protection. Such a coating also forms an excellent dielectric.

When using electrolytes of sea water or synthetic solutions of these salts as defined above in which the magnesium and calcium ion content is at least equal to that found in sea water and those electrolytes containing a concentration of magnesium and calcium ions sufficient to cause plating action when operating under the conditions delineated within the area of the graphs A to E inclusive, it is interesting to note the calcium and magnesium values in the electrocoatings which have been formed. These values are approximately as follows: Graph A has a magnesium equivalent of about 31% and a calcium equivalent of about 4%. On the other hand, graph E has a magnesium equivalent of about 2% and a calcium equivalent of about 34%. Graph C has a magnesium and calcium equivalent of approximately 15 and 18%, respectively. Graph B has values somewhere between those of graph A and C and graph D has values somewhere between graph C and D. Because of difficulty in separately analyzing these two elements of the alkaline-earth group, applicant does not wish to be limited to a definition of these curves in terms of either chemical content but he prefers to define the electrocoatings formed in terms of the physical characteristics as herein discussed. It should be noted that when operating as described a non-metallic coating can be formed which has characteristics approximating those of Fig. 5 or any variation thereof such as the poor deposits illustrated in Fig. 3 and Fig. 4.

In those instances wherein it is desired to coat a continuous wire, rod or strip wherein such wire, rod or strip is to be coated at a rate up to 600 feet per minute, my method may be carried out by utilizing an electrolyte temperature of 80 degrees C. and a current density of 10 amperes or more per square foot. A coating bath of sufficient extent to permit immersion of the article being coated for about six seconds would be sufficient to form a highly useful non-metallic coating of the type described. If, for example, it were desired to form such a non-metallic coating in three seconds, an electrolyte temperature of 90 degrees C. and a current density of 20 amperes per square foot could be utilized. At the higher current densities excellent "flash-type" coatings have been formed in as short a time as 1½ seconds.

This application is a continuation of my co-pending application Serial No. 733,213 filed Mar. 7, 1947 (now abandoned), which in turn is a continuation-in-part of my co-pending application Serial No. 526,621 filed Mar. 15, 1944 (now abandoned).

I claim:

1. The process of producing a two component protective coating on a metal surface which comprises the steps of submerging that part of the metal surface to be coated in an aqueous electrolyte, maintaining said part of the metal surface cathodic, maintaining the effective current density on the cathodic metal surface greater than 0.4 ampere per square foot, maintaining the cation content of said electrolyte to consist essentially of magnesium ions, other alkaline earth ions, and ions of an alkali in sufficient quantity to cause plating action to occur, maintaining the pH factor of said electrolyte within the range

between the limits of 4.0 and 9.5, and maintaining the temperature of the electrolyte below the boiling point under the operating conditions and within the range expressed by the equations  $T=34 \log_{10} X+30$  and  $T=34 \log_{10} X+70$ , where T is the temperature in degrees centigrade and X is the effective current density on the cathodic metal surface in amperes per square foot.

2. The process of producing a protective coating on a metal surface which comprises the steps of immersing that part of the metal surface to be coated in an electrolyte, maintaining said part of the metal surface cathodic, maintaining the cathodic current density greater than 0.4 ampere per square foot, maintaining the cation content of said electrolyte to consist essentially of the ions of magnesium, calcium and sodium in concentrations at least equal to those found in sea water of each of said elements and a sulfate ion concentration substantially equivalent to the cation content, maintaining the pH factor of said electrolyte between the limits of 4.0 and 9.5, and maintaining the temperature of the electrolyte below the boiling point under the operating conditions and within the range defined by the equations  $T=34 \log_{10} X+30$  and  $T=34 \log_{10} X+70$ , where T is the temperature in degrees centigrade and X is the cathodic current density in amperes per square foot.

3. The process of producing a protective coating on a metal surface which comprises the steps of immersing that part of the metal surface to be coated in an electrolyte, maintaining said part of the metal surface cathodic, maintaining the current density at the cathode greater than 0.4 ampere per square foot, maintaining the cation content of said electrolyte so as to consist essentially of the ions of magnesium, calcium and sodium in concentrations at least equal to those found in sea water of each of said elements and a chloride ion concentration substantially equivalent to the cation content, maintaining the pH factor of said electrolyte within the range between the limits of 4.0 and 9.5, and maintaining the temperature of the electrolyte below the boiling point under the operating conditions of pressure and ion concentration and within the range defined by the equations  $T=34 \log_{10} X+30$  and  $T=34 \log_{10} X+70$ , where T is the temperature in degrees centigrade and X is the current density at the cathode in amperes per square foot.

4. The process of producing a protective coating on a metal surface which comprises the steps of immersing that part of the metal surface to be coated in an electrolyte, maintaining said part of the metal surface cathodic, maintaining the cathodic current density greater than 0.4 ampere per square foot, maintaining the cation content of said electrolyte to consist essentially of the ions of magnesium, calcium and sodium in concentrations at least equal to those found in sea water of each of said elements and a nitrate ion concentration substantially equivalent to the cation content, maintaining the pH factor of said electrolyte between the limits of 4.0 and 9.5, and maintaining the temperature of the electrolyte below the boiling point under the operating conditions and within the range defined by the equations  $T=34 \log_{10} X+30$  and  $T=34 \log_{10} X+70$ , where T is the temperature in degrees centigrade and X is the cathodic current density in amperes per square foot.

5. The process of producing a protective coating on a metal surface which comprises the steps of immersing that part of the surface to be coated

in an electrolyte, maintaining said part of the metal surface cathodic, maintaining the cathodic current density greater than 0.4 ampere per square foot, maintaining the cation content of said electrolyte to consist essentially of the ions of magnesium, calcium and sodium in concentrations at least equal to those found in sea water of each of said elements and an anion content of chlorides, sulfates and nitrates, said anion concentration being substantially equivalent to the cation content, maintaining the pH factor of said electrolyte between the limits of 4.0 and 9.5, and maintaining the temperature of the electrolyte below the boiling point under the operating conditions and within the range defined by the equations  $T=34 \log_{10} X+30$  and

$$T=34 \log_{10} X+70$$

where  $T$  is the temperature in degrees centigrade and  $X$  is the cathodic current density in amperes per square foot.

6. The process of producing a protective coating on a metal surface which comprises the steps of immersing that part of the metal surface to be coated in an electrolyte, maintaining said part of the metal surface cathodic, maintaining the cathodic current density greater than 0.4 ampere per square foot, maintaining said electrolyte to comprise essentially an aqueous solution providing ions of magnesium and calcium to be electrolytically deposited, maintaining the pH factor of said electrolyte within the range between the limits of 4.0 and 9.5, and maintaining the temperature of the electrolyte below the boiling point under the operating conditions and within the range expressed by the equations

$$T=34 \log_{10} X+30$$

and  $T=34 \log_{10} X+70$ , where  $T$  is the temperature in degrees centigrade and  $X$  is the cathodic current density in amperes per square foot.

7. The process of producing a protective coating on a metal surface which comprises the steps of immersing that part of the surface to be coated in an electrolyte, maintaining said part of the metal surface cathodic, maintaining the cathodic current density greater than 0.4 ampere per square foot, maintaining said electrolyte to consist of an aqueous solution having as the essential plating components magnesium and calcium ions in sufficient quantities for plating action to occur, maintaining the pH factor of said electrolyte within the range between the limits of 4.0 and 9.5, and maintaining the temperature of the electrolyte below the boiling point under the operating conditions and within the range expressed by the equations  $T=34 \log_{10} X+30$  and  $T=34 \log_{10} X+70$ , where  $T$  is the temperature in degrees centigrade and  $X$  is the cathodic current density in amperes per square foot.

GEORGE C. COX.

#### REFERENCES CITED

The following references are of record in the file of this patent:

#### UNITED STATES PATENTS

| Number    | Name                | Date         |
|-----------|---------------------|--------------|
| 872,759   | Schoneberger et al. | Dec. 3, 1907 |
| 2,200,469 | Cox                 | May 14, 1940 |

#### FOREIGN PATENTS

| Number | Country       | Date    |
|--------|---------------|---------|
| 6,495  | Great Britain | of 1894 |